

Jan. 27, 1942.

C. E. NELSON

2,271,023

METHOD OF TREATING MAGNESIUM

Filed May 11, 1940



*Fig. 1*

INVENTOR  
Charles E. Nelson  
BY Griswold & Burdick  
ATTORNEYS

## UNITED STATES PATENT OFFICE

2,271,023

## METHOD OF TREATING MAGNESIUM

Charles E. Nelson, Midland, Mich., assignor to  
The Dow Chemical Company, Midland, Mich., a  
corporation of Michigan

Application May 11, 1940, Serial No. 334,593

7 Claims. (Cl. 75—67)

This invention relates to the treatment of magnesium. It more particularly concerns a method of treating commercial magnesium whereby it is rendered highly pure, or the magnesium in magnesium scrap, such as castings, alloys and the like, can be recovered in a highly pure state.

I have found that the presence of certain impurities in magnesium, even though these be present in very limited amounts, greatly accelerates the rate at which magnesium corrodes. For example, it is recognized that the presence of a small amount of iron in magnesium greatly accelerates the rate at which magnesium corrodes and may thus render it unsuitable for many commercial uses. The impurities nickel and copper affect the rate at which magnesium metal corrodes similarly.

To remove these impurities ordinarily present in the magnesium produced by present practices, it has heretofore been proposed to subject the magnesium to sublimation or distillation. However, I have observed that unless the metal being purified is subjected to repeated sublimation or distillation, as the case may be, the impurities are not generally removed to the extent that they no longer greatly accelerate the rate at which magnesium corrodes or otherwise adversely affect the properties of the metal. In some instances, even by repeated distillations or sublimations, the metal cannot be rendered satisfactorily pure.

It is, therefore, the principal object of the invention to provide a method of rendering magnesium so highly pure that the impurities no longer have substantially any adverse effect as regards the rate at which magnesium corrodes. Another object of the invention is to provide a method whereby magnesium can be rendered pure in a single operation. Other objects and advantages will be apparent as the description proceeds.

I have discovered that, if the magnesium to be purified is caused to vaporize in the presence of a metal selected from the group of metals consisting of lead, tin, bismuth, calcium, silicon, and antimony and thereafter passed through a filter bed of a refractory material selected from the group of refractories comprising the oxides and silicates of metals located above manganese in the electromotive force series of metals, impurities can be removed to the extent that the rate to which commercial magnesium corrodes is greatly reduced.

The invention then resides in the method

hereinafter fully described and particularly pointed out in the claims, the accompanying drawing and following description setting forth in detail a mode of carrying out the invention, such mode illustrating, however, but one of various ways in which the principle of the invention may be used.

In said drawing:

Fig. 1 is a sectional view in elevation of the apparatus;

Fig. 2 is a top plan view of said apparatus.

In the drawing an upright cylindrical iron retort 1 is shown closed at the bottom and is provided at the top end with a flange 2, to which is attached a gasket sealed head 3 by means of suitable bolts 4. Condenser 5, in the form of a section of iron pipe closed at its lower end is attached centrally to the interior side of head 3 and extends into the retort. Externally of the retort a cooling water inlet 6 and water outlet 7 communicate with the interior of the condenser 5. A mass of purified condensed magnesium 8 is shown clinging to the condenser 5. A vacuum connection 9 communicates through

head 3 with the interior of the retort and provides a means whereby the retort may be connected to a vacuum pump (not shown) and held under reduced pressure. A cooling coil 10 intimately attached to head 3 (as by welding)

30 encircles the head directly above gasket 11 and serves to prevent the gasket from becoming over-heated. Internally of the retort a removable iron charge container 12 partially filled with a solid charge 13 consisting of a quantity of im-

35 pure magnesium and a suitable metal added to effect the purification of the magnesium rests on the bottom of the retort. A shallow perforate metal basket 14, which engages the top rim of container 12, is suspended from charge con-

40 tainer 12 by means of flange 15. The perforate basket is shown filled with granular particles of a refractory material, designated generally by numeral 16, which acts as a filter through which the vaporized magnesium passes. A perforate

45 cover 17 is provided for basket 14 and serves to confine the filter bed during the purifying operation. As a means of heating the retort electrical leads 18 are connected to a resistance wire 19 which encircles the lower portion of the retort. A suitable insulating material 20 surrounds the retort and serves to protect it from excessive heat loss due to radiation.

In carrying out the method of the invention the iron charge container 12, filled with charge 55 13, consisting of impure magnesium and the

added purifying metal is lowered into the retort through the open end. The perforate metal basket containing the refractory material which is to act as the filter is then positioned on top of the charge container. After the cover 17 has been placed upon the perforate basket 14, the retort is closed by bolting the flanged head 3 in place. Cooling water is then started through the lines 6 and 7 and through coil 10 while vacuum is applied to exhaust the interior of the retort of gases to line 9. When the desired degree of vacuum is obtained electrical current is supplied to the resistance wire 19 through electrical leads 18 to heat the retort, care being taken in the meantime to maintain the vacuum. The impure magnesium as well as the added metal rapidly melts and as the magnesium vapor forms it passes through filter bed of refractory material 16 which exerts a further purifying action and finally collects and condenses on the cold surface of condenser 5 where it adheres in the form of compact crystals. After such time has elapsed as will indicate that substantially all the magnesium has been distilled off the current may be shut off, the vacuum broken and the flanged head 3 detached from the retort. The magnesium crystals can then be scraped from the condenser. Additional impure magnesium may be immediately added to the charge container without removing the residue therefrom and the process of purifying the metal continued. However, it is generally preferable to renew the refractory contained in the perforate metal basket after each purifying operation since it tends to crumble and become powdery under the temperature conditions of operation.

As afore-mentioned, the metals suitable for use are the metals selected from the group of metals consisting of lead, tin, bismuth, calcium, silicon, and antimony. If desired, mixtures of these metals may be suitably employed. For example, a particularly effective mixture consists of tin and lead. In general the amount of such metal to employ to effect the removal of undesirable impurities is from 10 to 50 per cent or more by weight, based upon the weight of the impure magnesium, and preferably between 25 and 35 per cent. It is unnecessary to remove the residue, consisting mainly of the added metal, from the charge container after every run, since in practice it has been found that as many as 20 or more charges of impure magnesium may be purified with but a single addition of the purifying metal.

The filtering materials to be employed are the refractories consisting of oxides and silicates located above manganese in the electromotive force series of metals. Examples of such refractories are calcium silicate, barium oxide, aluminum oxide and the like. If desired mixtures of these metals may be employed. Complex mixtures of oxides and silicates have also been found to be highly effective. For example, a material preferred because of its especial effectiveness is the ordinary rock wool or mineral wool of commerce which is obtained by mechanically processing naturally occurring rock compositions consisting mainly of silicon oxide, alumina, and magnesia. Another silicate useful for the purpose at hand is exploded mica. The materials are preferably employed in the form of granular particles or, in the case of rock wool, as fibrous material, and in this form give a filter bed that is readily permeable to the magnesium vapor. The filter bed made of these materials should be made of  $\frac{1}{2}$  to 2 inches or more in thickness to produce the

most effective purification. As afore-mentioned it is generally desirable to renew the filter bed after each run since the materials tend to become soft and crumble easily after being heated to the temperature required for the operation of the process.

The purifying effect produced by passing the vaporized metal through a bed of these refractories is not entirely due to a mechanical filtering action, but is also due to some chemical action between the impurities and the refractory. This is evidenced by the fact that by merely adding a quantity of rock wool to a charge of impure magnesium, and thereafter distilling or subliming the magnesium, a product of greater purity is obtained than can be obtained by just distilling impure magnesium. Thus merely bringing the vaporized magnesium into contact with the filtering or purifying medium suffices to yield a purified condensate.

It is usually desirable to operate under relatively high vacuum, as for example, less than 2 millimeters of mercury, and preferably below 0.2 of a millimeter, since under such highly reduced pressure the purified magnesium condenses out in the form of a dense compact mass rather than in the form of long needle-like crystals. Condensation in a dense compact form is desirable because relatively little surface area is exposed to oxidation when the metal is later remelted or the like, in comparison with the area exposed when a needle-like crystal structure is produced. Operating at highly reduced pressure offers the additional advantage that the temperature required to effectively carry out the process is such that the apparatus may be constructed of readily available iron or steel without any danger of destruction due to the high temperature necessary if the purifying operation is carried out at higher pressure. If desired, a suitable inert gas such as helium, argon, and the like may be introduced into the retort to prevent destructive attack by air or other gases upon the purified metal, although under the preferred vacuum conditions such procedure is unnecessary.

The temperature to be employed in the distillation or sublimation may, of course, be varied quite widely, as for example, between about 500° to 800° C., depending, however, upon the degree of vacuum employed. At 0.05 millimeter pressure of mercury a temperature of 700° C. has been found highly satisfactory. It is preferable that the magnesium be caused to vaporize at such a temperature that the added metal melts in the presence of the magnesium vapor.

The time required to purify a batch of metal also depends upon the amount of heat supplied to the metal as well as the pressure employed. In a retort such as illustrated, 16 inches in diameter, it is possible to distill off from three to four pounds of magnesium per hour by holding the temperature at about 700° C. and the pressure at 0.05 millimeter.

A generally desirable combination to employ, because of the high degree of purity of the product obtained, is from 15 to 20 per cent by weight of lead in combination with a filter composed of rock wool.

This application is a continuation-in-part of my application Serial No. 257,924, filed February 23, 1939.

Other modes of applying the principle of my invention may be employed instead of those explained, change being made as regards the method herein disclosed, provided the step or steps stated

by any of the following claims or the equivalent of such stated step or steps be employed.

I therefore particularly point out and distinctly claim as my invention:

1. The method of producing substantially pure magnesium comprising introducing impure magnesium into direct contact with from 10 to 50 per cent by weight of a metal selected from the group of metals consisting of lead, tin, calcium, bismuth, antimony, and silicon, applying heat so as to cause the metals to alloy, continuing the application of heat so as to cause the magnesium to vaporize, and thereafter passing the magnesium vapor through a filter bed of a refractory material selected from the group of refractory materials consisting of the oxides and silicates of the metals located above manganese in the electromotive series of metals.

2. The method of producing substantially pure magnesium comprising bringing impure magnesium into direct contact with from 25 to 35 per cent by weight of a metal selected from the group of metals consisting of lead, tin, calcium, bismuth, antimony, and silicon, applying heat so as to cause the metals to alloy, continuing the application of heat so as to vaporize the magnesium while maintaining the metals under reduced pressure, and thereafter passing magnesium vapor through a filter bed comprising a refractory material selected from the group of refractory materials consisting of the oxides and silicates of the metals located above manganese in the electromotive series of metals.

3. The method of producing substantially pure magnesium comprising heating an alloy consisting of magnesium and from 10 to 50 per cent by weight of at least one of the metals selected from the group of metals consisting of lead, tin, calcium, bismuth, antimony, and silicon so as to cause the magnesium contained in the alloy to vaporize, passing the magnesium vapor through a filter bed of a refractory material selected from the group of refractory materials consisting of the oxides and silicates of the metals located above manganese in the electromotive series of metals.

4. The method of producing substantially pure magnesium comprising heating an alloy under reduced pressure, consisting of magnesium and from 10 to 50 per cent of at least one of the metals

selected from the group of metals consisting of lead, tin, calcium, bismuth, antimony, and silicon so as to cause the magnesium contained in the alloy to vaporize, passing the magnesium vapor through a filter bed of a refractory material selected from the group of refractory materials consisting of the oxides and silicates of the metals located above manganese in the electromotive series of metals.

5. The method of producing substantially pure magnesium comprising heating an alloy consisting of magnesium and from 10 to 50 per cent by weight of at least one of the metals selected from the group of metals consisting of lead, tin, calcium, bismuth, antimony, and silicon so as to cause the magnesium contained in the alloy to vaporize and thereafter bringing the magnesium vapor into contact with a refractory material selected from the group of refractory materials consisting of the oxides and silicates of the metals located above manganese in the electromotive series of metals without causing the magnesium vapor to condense.

6. The method of producing substantially pure magnesium comprising heating an alloy consisting of magnesium and from 25 to 35 per cent by weight of at least one of the metals selected from the group of metals consisting of lead, tin, calcium, bismuth, antimony, and silicon so as to cause the magnesium contained in the alloy to vaporize, bringing the magnesium vapor into contact with a refractory material selected from the group of refractory materials consisting of the oxides and silicates of the metals located above manganese in the electromotive series of metals without condensing said magnesium vapor, and thereafter separately condensing the magnesium vapor.

7. The method of producing substantially pure magnesium comprising bringing impure magnesium into direct contact with from 25 to 35 per cent by weight of lead, applying heat so as to alloy the magnesium and lead, continuing the application of heat so as to vaporize the magnesium while holding the metals under reduced pressure, passing the magnesium vapor through a filter bed comprising rock wool, and thereafter condensing the magnesium.

CHARLES E. NELSON.